

## UNITED STATES PATENT OFFICE

2,248,185

## HEAT TREATMENT OF ALUMINUM BASE ALLOYS

Joseph A. Nock, Jr., Tarentum, Pa., assignor to  
Aluminum Company of America, Pittsburgh,  
Pa., a corporation of Pennsylvania

No Drawing. Application July 12, 1939,  
Serial No. 283,995

8 Claims. (Cl. 148—21.1)

This invention relates to aluminum base alloys containing zinc, magnesium, copper, and manganese, and is more particularly concerned with the treatment of such alloys to prevent corrosion thereof. By the term aluminum base alloys, I mean alloys containing more than 50 per cent aluminum.

A large number of aluminum base alloys are susceptible to improvement in tensile strength, yield strength, hardness, and other physical properties by various thermal treatments. One of the most common of these treatments, which is usually employed in combination with a subsequent precipitation or age-hardening treatment and is often referred to as a solution heat-treatment, consists in subjecting the alloy to a temperature and for a time sufficient to cause solution of a substantial quantity of the soluble elements of the alloy but below the fusion temperature of the alloy's lowest melting point constituent. These elements then may be retained in solution by a relatively rapid cooling or quenching to room temperature. Following this solution heat-treatment and quenching, the strength, hardness and other properties of some aluminum alloys may be further improved if the alloys are permitted to stand or age for a few days, or are artificially aged at a temperature of about 200° F. to 350° F. for a shorter period of time.

Among the alloys which are susceptible to improvement by solution heat-treatment, quenching, and artificial aging are the aluminum base alloys containing zinc, magnesium, copper, and manganese. Such alloys are heated to a temperature between about 850° F. and 1000° F. and maintained at that temperature for a period of from about 5 minutes to about 10 hours in order to place a substantial portion of the soluble constituent of the alloy in solution, and, following quenching to normal temperature, they are aged usually for about 2 to 30 hours at a temperature between about 200° F. and about 350° F. These alloys develop high tensile and yield strengths and other desirable properties when treated as above described. However, unless they are very rapidly or drastically cooled, following age-hardening they sometimes develop a susceptibility to a type of intergranular corrosion when exposed to corrosive conditions. This attack is believed to be due to the precipitation within the metal of a portion of the soluble alloying constituent and to galvanic action caused by the difference in potentials between the precipitated phase and the metal itself. This type of corrosion is accelerated when articles of these alloys are sub-

jected to stress, either internal or external in source, which tends to fracture the alloy, thereby exposing fresh surfaces to corrosive agents. Such corrosion in alloys of this type can be substantially prevented if the alloy article is very rapidly or drastically quenched in cold water following solution heat-treatment, but this procedure is often impractical because it is apt to produce distortion or warpage of the article.

10 The object of my invention is to improve the resistance to corrosion of articles of thermally treated aluminum base alloys containing zinc, magnesium, copper, and manganese, and especially of such articles which are subjected in use to stress. More particularly, the object of the invention is to provide such a method for improving the resistance to corrosion of articles of alloys of the class above described, following their solution heat-treatment, which avoids the distortion resulting from the drastic quenching or rapid cooling of such articles. The specific object of my invention is to provide a method for improving the resistance to corrosion of such articles of aluminum base alloys containing zinc, 25 magnesium, copper, and manganese which have been subjected to solution heat-treatment and have been cooled at a relatively slow rate and subsequently artificially aged. Other objects will appear in the following description of the invention.

30 My invention is predicated upon the discovery that the resistance to corrosion of solution treated and relatively slowly quenched articles of aluminum base alloys containing zinc, magnesium, copper, and manganese may be increased if they are given a comparatively low temperature heat-treatment following the normal artificial age-hardening thereof. This treatment preferably is carried out by heating the articles at the termination of their artificial age-hardening period for a duration of between about 15 minutes and about 2 hours at a temperature of about 350° F. to 450° F. The articles then may be cooled to room temperature in any convenient manner, as, for instance, by natural cooling or by quenching, without distortion of their shape. This treatment may be practiced at very little expense and is adapted to be carried out in the heat-treating equipment commonly used.

40 The above described method has been found to be particularly adapted to aluminum base alloys containing between about 3 per cent and about 10 per cent zinc, between about 0.75 per cent and about 4 per cent magnesium, between 45 about .05 per cent and about 3 per cent copper,

and between about 0.1 per cent and about 1.5 per cent manganese. Various amounts of other elements also may be present to modify or improve certain properties of the alloys, as for example, titanium, vanadium, zirconium, chromium, cobalt, tungsten, columbium, or tantalum.

In a specific application of my invention, I have tested specimens of an alloy containing 5.46 per cent zinc, 2.21 per cent magnesium, 1.51 per cent copper, 0.42 per cent manganese, 0.28 per cent iron, 0.17 per cent silicon, and 0.09 per cent titanium, the remainder of the alloy being aluminum. These specimens were given a solution heat-treatment often employed for this alloy at a temperature of 900° F. for a period of between 15 and 20 minutes. Some of the specimens were then very rapidly quenched in cold water and the others were more slowly cooled by a high velocity air blast. Although all of the specimens were cooled rapidly enough to effect a supersaturated solution of the alloying constituent in the metal at room temperature, the specimens which had been drastically quenched were distorted and twisted by their very rapid cooling, while the specimens which had been cooled at a relatively slow rate retained their shape. All specimens were then given an artificial aging treatment for 8 hours at a temperature of 275° F., following which it was found that there was no material difference between the strength and elongation of the specimens which had been very rapidly cooled and of those which had been more slowly cooled from the solution temperature.

These specimens were then exposed to corrosive conditions. More specifically, they were repeatedly subjected to short periods of immersion in an 0.9 normal sodium chloride aqueous solution containing 0.3 per cent hydrogen peroxide and to short intervening periods of exposure to the atmosphere. During this procedure some of the specimens were subjected to stress equivalent to 75 per cent of the yield strength of the alloy in order that their resistance to stress corrosion might be determined. This repeated cycle of

alternating immersion of the specimens into the solution and exposure to the atmosphere was continued for a period of 48 hours, after which the specimens were tested for the usual physical properties, as hereinafter disclosed.

The tests showed that the specimens which had been relatively slowly cooled from the solution heat-treating temperature had suffered much greater losses in properties due to corrosion than had those which had been very rapidly quenched; and of the slowly cooled specimens, those which had been subjected to stress during exposure to corrosive conditions showed a much greater loss in properties than did the unstressed specimens. These observations indicate that relatively slowly cooled objects of the particular alloy have a much lower resistance to corrosion, particularly if they are subjected to stress while exposed to corrosive conditions, than the drastically quenched objects.

Some of the age-hardened specimens which had been relatively slowly quenched and aged for 8 hours at 275° F. were then heated for ½ hour at temperatures of 375°, 400°, and 425° F. These were exposed to the corrosive conditions described above, some of the specimens being subjected to stress during exposure and the others being unstressed. Following 48 hours of alternating exposure to the salt solution and to the atmosphere, the specimens were tested. The tests showed that the percentage loss of properties was not appreciably greater in the slowly quenched specimens which had been given a secondary relatively low temperature heat-treatment than it had been in the drastically quenched specimens, indicating that the resistance to corrosion of the slowly cooled specimens, even under stress, was substantially equivalent to that of the drastically cooled specimens as a result of the above described thermal treatment subsequent to age-hardening.

The test results are tabulated herewith. The numbers preceding the test results are identified at the end of the table.

| Properties of heat-treated, quenched, and aged articles |                                  |                         | Percentage loss in properties following exposure to corrosion |                       |                      |                       |
|---------------------------------------------------------|----------------------------------|-------------------------|---------------------------------------------------------------|-----------------------|----------------------|-----------------------|
| Tensile strength                                        | Yield strength                   | Elongation              | Unstressed                                                    |                       | Stressed             |                       |
|                                                         |                                  |                         | Tensile strength                                              | Elong.                | Tensile strength     | Elong.                |
| Lbs./sq. in.<br>1 74,610<br>3 75,900                    | Lbs./sq. in.<br>64,750<br>64,000 | Percent<br>12.8<br>14.0 | Percent<br>-4<br>-10                                          | Percent<br>-43<br>-66 | Percent<br>-5<br>-24 | Percent<br>-49<br>-87 |

| Properties of heat-treated, quenched, and aged articles following secondary heat-treatment |                                            |                             | Percentage loss in properties following exposure to corrosion |                              |                           |                              |
|--------------------------------------------------------------------------------------------|--------------------------------------------|-----------------------------|---------------------------------------------------------------|------------------------------|---------------------------|------------------------------|
| Tensile strength                                                                           | Yield strength                             | Elongation                  | Unstressed                                                    |                              | Stressed                  |                              |
|                                                                                            |                                            |                             | Tensile strength                                              | Elong.                       | Tensile strength          | Elong.                       |
| Lbs./sq. in.<br>1 71,690<br>4 70,630<br>3 67,530                                           | Lbs./sq. in.<br>63,900<br>62,860<br>57,350 | Percent<br>10<br>10<br>10.5 | Percent<br>-5<br>-6<br>-3                                     | Percent<br>-40<br>-50<br>-16 | Percent<br>-6<br>-6<br>-4 | Percent<br>-40<br>-50<br>-31 |

<sup>1</sup> Very rapidly quenched from solution heat-treatment temperature.

<sup>2</sup> Relatively slowly quenched from heat-treatment temperature.

<sup>3</sup> Relatively slowly quenched from heat-treatment temperature and treated at 375° F. following age-hardening.

<sup>4</sup> Relatively slowly quenched from heat-treatment temperature and treated at 400° F. following age-hardening.

<sup>5</sup> Relatively slowly quenched from heat-treatment temperature and treated at 425° F. following age-hardening.

While my invention has been described in connection with the treatment of a specific alloy, it may be practiced with advantage to increase the resistance to stress corrosion of articles of other aluminum base alloys containing zinc, magnesium, copper, and manganese which have been cooled from the solution heat-treatment temperature at a relatively slow rate and subsequently age-hardened; and the invention may be utilized with particular advantage where it is desirable to avoid distortion of the shape of articles of such alloys which are to be subjected to solution heat-treatment and age-hardening.

I claim:

1. A method of heat-treating an aluminum base alloy containing zinc, magnesium, copper, and manganese which comprises heating the alloy at a temperature and for a time sufficient to place a substantial portion of its soluble constituent in solution, quenching the alloy, artificially aging the alloy, and subsequently heating the alloy between 350° F. and 450° F. for from about 15 minutes to about 2 hours.

2. A method of heat-treating an aluminum base alloy containing zinc, magnesium, copper, and manganese which comprises heating the alloy between 850° F. and 1000° F. for from 5 minutes to 10 hours, quenching the alloy at a relatively slow rate, aging the alloy between 225° F. and 350° F. for a period of between 2 and 30 hours, and subsequently heating the alloy at a temperature of between 350° F. and 450° F. for a period of from about 15 minutes to about 2 hours.

3. A method of heat-treating an aluminum base alloy containing from about 3 per cent to about 10 per cent zinc, from about 0.75 per cent to about 4 per cent magnesium, from about 0.5 per cent to about 3 per cent copper, and from about 0.1 per cent to about 1.5 per cent manganese, which method comprises heating said alloy at a temperature and for a time sufficient to place a substantial portion of the soluble constituent thereof in solution, quenching the alloy at a relatively slow rate, artificially aging the alloy, and subsequently heating the alloy at a temperature of between 350° F. and 450° F. for a period of from about 15 minutes to about 2 hours.

4. A method of heat-treating an article of aluminum base alloy, said alloy containing zinc, magnesium, copper, and manganese, which comprises heating the article at a temperature and for a time sufficient to place a substantial portion of the soluble constituent of said alloy in solution, quenching the article at a rate suffi-

ciently slow to avoid distortion of the shape of the article and sufficiently rapid to retain a substantial portion of the constituent of said alloy in solid solution, artificially aging the article, and subsequently heating the article between 350° F. and 450° F. for from about 15 minutes to about 2 hours.

5. A method of heat-treating an aluminum base alloy containing zinc, magnesium, copper, and manganese, which comprises heating the alloy at a temperature and for a time sufficient to place a substantial portion of its soluble constituent in solution, air quenching the alloy, artificially aging the alloy, and subsequently heating the alloy between 350° F. and 450° F. for a period of from about 15 minutes to about 2 hours.

10 6. The method of increasing corrosion resistance of an aluminum base alloy containing zinc, magnesium, copper, and manganese, which has been relatively slowly cooled from the solution heat-treatment temperature and artificially age-hardened, which method comprises heating said alloy to a temperature of between about 350° F. and about 450° F. and maintaining the alloy at said temperature for a period of about 15 minutes to about 2 hours.

15 7. In the treatment of an aluminum base alloy containing zinc, magnesium, copper, and manganese to increase its strength and hardness by heating said alloy at a temperature and for a time sufficient to place a substantial portion of the soluble constituent thereof in solution, cooling the alloy at a relatively slow rate, and artificially aging the alloy, the subsequent step of heating said alloy for a period of from about 15 minutes to about 2 hours at a temperature of between about 350° F. and 425° F. to improve the resistance of said alloy to corrosion.

20 8. The method of increasing the strength and hardness of an article of aluminum base alloy containing zinc, magnesium, copper, and manganese, said method being characterized by a resulting increase in the resistance of the article to corrosion and the absence of substantial distortion to the shape of the article, which method comprises heating said article at a temperature and for a time sufficient to place a substantial part of the soluble constituent of said alloy in solution, cooling the article at a relatively slow rate, artificially aging the article, and then heating the article at a temperature of between about 350° F. and 450° F. for a period of from about 15 minutes to about 2 hours.

JOSEPH A. NOCK, JR.